

June 4, 1940.

S. E. SHEPPARD ET AL

2,203,659

PHOTOGRAPHIC ANTIHALATION LAYER

Filed April 12, 1939

FIG.1.



FIG. 2.



FIG. 3.



Samuel E. Sheppard  
Robert C. Houck  
INVENTORS

BY

*Newton M. Perrins*  
*R. Frank Smith*

ATTORNEYS

Patented June 4, 1940

2,203,659

# UNITED STATES PATENT OFFICE

2,203,659

## PHOTOGRAPHIC ANTHALATION LAYER

Samuel E. Sheppard and Robert C. Houck, Rochester, N. Y., assignors to Eastman Kodak Company, Rochester, N. Y., a corporation of New Jersey

Application April 12, 1939, Serial No. 267,479

9 Claims. (Cl. 95—9)

This invention relates to antihalation layers for photographic films.

This application is a continuation-in-part of our application Serial No. 102,546, filed September 25, 1936.

The purpose of providing films with antihalation layers is well known in the photographic art. When a photographic film is exposed, there is a tendency for light to be reflected from the surface of the film support or other layer of the film and to produce on the sensitive emulsion layer, according to its intensity, halos surrounding brighter parts of the image. This effect is known as halation and it is customary to coat the rear surface of the support with a coloring material which absorbs the light and prevents a reflection onto the sensitive layer. Where the film is to be used as a transparency, the coloring matter designed for antihalation purposes must, of course, be removed.

It is obvious that the coloring matter used for this purpose should be removed as completely as possible during processing of the film. Dyes used for this purpose sometimes have a tendency to stain the support or other layers of the film and to be retained in the film after processing. Some dyes which are readily removed in an alkaline solution, such as a photographic developer, have a tendency to discolor the developer to such an extent that it is rendered useless for further development. It is desirable to maintain the developing solution in a pure condition so that it may be used to develop large amounts of film.

It is therefore an object of the present invention to provide an antihalation layer having a dye which is readily decolorized in the processing baths. It is a further object to provide an antihalation dye which is removable in an acid solution such as a fixing bath, but not in a developer solution. It is a still further object to provide a new class of antihalation dyes.

These objects are accomplished by incorporation in a gelatin layer, applied to the film, a dye or dyes which are analogues of murexide.

We may use murexide itself as well as analogous compounds, and by the term "analogues of murexide," we include murexide itself as well as analogous compounds.

In the accompanying drawing we have shown a number of enlarged sectional views of photographic film coated with antihalation dyes according to our invention. In the drawing:

Fig. 1 is a sectional view of a film having an antihalation layer on the rear surface of the support.

Fig. 2 is a sectional view of a film having an antihalation layer between the emulsion layer and the support, and

Fig. 3 is a sectional view of a film having an antihalation layer coated over the emulsion layer.

We have found that a number of dyes including analogues of murexide, as well as murexide itself, may be incorporated in gelatin to give a purple-red color such that the gelatin is suitable for use as antihalation backings. These dyes have the property of discharging readily and completely in ordinary acid fixing baths having a pH of about four.

The dyes which we use have the general formula:



where R and R' represent the atoms necessary to complete a carbocyclic or heterocyclic ring, and X represents an alkali metal or alkaline earth radical, such as sodium, potassium, or ammonium, or nickel.

The principal compound of this group which we contemplate using is murexide, which is the ammonium salt of purpuric acid, and has the following constitution:



The color discharge when the gelatin layer dyed with this compound is subjected to an acid fixing bath is probably associated with the formation of the keto-isomer of purpuric acid which is decomposed by hydrolysis to alloxan and uramyl. The structure of this compound (purpuric acid) may be represented as follows:



Other dyes which we contemplate using are the following: Rubazonic acid:



Diketohydrindylidenediketohydrindamine:



## Diketohydrindylideneuramil:



## Diketohydrindylidene - keto - phenylmethyl - pyrazolamine



15 The compound murexide may be produced by the condensation of alloxan and uramil in an alkaline solution in the usual manner. The other compounds listed above may be produced by 20 treating the carbocyclic or heterocyclic nucleus with hydroxylamine, reducing the oxime formed in this way and condensing the reduction product with the original or a different ring compound. For example, rubazonic acid may be produced by 25 treating 1-phenyl-3-methyl-pyrazoledione with hydroxylamine and reducing the oxime formed in this way. The reduction product is then condensed with an equimolecular amount of the original ring compound to produce rebazonic acid. The equations for this reaction may be represented as follows:



50 In a similar manner the compound diketohydrindylidenediketohydrindamine is produced by condensing 2 molecules of triketohydrindine; the compound diketohydrindylideneuramil is produced by condensing a molecule of uramil with a molecule of triketohydrindine and the compound diketohydrindylidene - keto - phenylmethyl - pyrazolamine is produced by condensing a molecule of 1-phenyl-3-methyl-pyrazolamine with a molecule of triketohydrindine.

55 It is not known whether these compounds exist in the keto or the enol form in every case, but it

is now understood that there is a virtual tautomerizing or resonance in the chromophore chain which would mean an oscillation between the enolic and ketonic forms, indicated as follows:



60 The color obtained when an analogue of murexide is added to gelatin is dependent on several factors, including the ash content of the gelatin, and the alkali used to adjust the pH of the gelatin solution. In general, it may be said that with high ash gelatin, color is produced either in acid or alkaline solution, regardless of the alkali used to adjust the pH. With low ash gelatin, flocculation occurs, especially in alkaline solution, when the pH is adjusted with a strong inorganic alkali, while a uniform color is produced in either acid or alkaline solution in which the pH is adjusted with an organic alkali. This is indicated by the following table:

|                     | Acid solution                                                                                           | Alkaline solution                                                                                       |
|---------------------|---------------------------------------------------------------------------------------------------------|---------------------------------------------------------------------------------------------------------|
| High ash gelatin... | Orange color.....                                                                                       | Orange color.                                                                                           |
| Low ash gelatin...  | NaOH-flocculation.....<br>NH <sub>4</sub> OH-flocculation.....<br>Triethanolamine.....<br>purple color. | NaOH-flocculation.....<br>NH <sub>4</sub> OH-purple color.....<br>Triethanolamine.....<br>purple color. |

65 The high ash gelatin may be an original undeashed photographic gelatin containing from 1% to 2% ash. The low ash gelatin may be deashed gelatin originally obtained by lime processing, or an acid processed gelatin, as described in Sheppard and Hudson U. S. Patent No. 2,101,877, December 14, 1937. De-ashed or acid processed gelatin usually has an ash content of less than 0.2%.

70 The following examples, which are illustrative only, indicate methods of forming antihalation layers according to our invention:

## Example 1

75 A quantity of deashed gelatin having an ash content of about 0.02% was adjusted to a pH of 7.3 with triethanolamine. Murexide was added in the amount of 1% of the weight of gelatin solution, and the colored mixture coated on a support. The gelatin coating had a reddish-purple color which it retained on drying, and was suitable for use as an antihalation layer.

## Example 2

80 1.25 grams of the potassium salt of diketohydrindylideneuramil were dissolved in 50 cc. of water, and this solution was added to a solution of 7 grams of deashed gelatin in 50 cc. of water, the pH of the gelatin solution having been adjusted to 8.9 with ammonium hydroxide. This mixture was coated on a glass plate having a cellulose nitrate coating, and permitted to dry. The film thus formed had a reddish-purple color suitable for use as an antihalation backing.

85 The antihalation layers made according to our invention may be used in various ways to coat photographic film. In the accompanying drawing we have shown in Fig. 1 a sectional view of the usual film construction in which 10 represents a transparent support of cellulose nitrate, cellulose acetate or other suitable material coated with an emulsion layer 11. On the opposite side of the support 10 there is coated a gelatin layer 12

containing one of the analogues of murexide used according to our invention. Fig. 2 represents another type of film in which the antihalation layer 12 is coated between the support 10 and the emulsion layer 11. Fig. 3 represents a further type of film in which the antihalation layer 12 is coated over the emulsion layer 11, which is coated on the support 10. This latter type of film is designed for use in exposure of the sensitive emulsion layer 10 through the support, and in this type as well as in the other types of film, it is highly desirable to remove the antihalation layer during the processing of the film. The colored layer may also serve as a filter layer, in which case the emulsion layer is exposed through the colored layer.

It is to be understood that the examples of the dye compounds and the methods of using them incorporated in the above specification are by way of illustration only and that our invention is to be taken as limited only by the scope of the appended claims.

We claim:

1. A photographic element comprising a support, a sensitive emulsion layer thereon, and a layer of unsensitized gelatin thereon uniformly colored with a compound of the general formula:



where R and R' represent the atoms necessary to complete a ring structure and X represents an alkali metal radical.

2. A photographic element comprising a support, a sensitive emulsion layer thereon, and a layer of unsensitized gelatin thereon uniformly colored with murexide.

3. A photographic film comprising a transparent support, a gelatino-silver halide emulsion layer on said support, and a layer of unsensitized gelatin on said support containing murexide, the emulsion layer being located between the source of exposing light and the unsensitized gelatin layer.

4. A photographic film comprising a transparent support, a sensitive emulsion layer on one side of said support, and on the opposite side of said support a layer of unsensitized gelatin uniformly colored with a compound of the general formula:



wherein R and R' represent the atoms necessary to complete a ring structure and X represents an alkali metal radical.

5. A photographic element comprising a transparent support, a gelatino-silver halide emulsion layer on one side of said support, and on the opposite side of said support a layer of gelatin uniformly colored with murexide.

6. The method of forming a photographic antihalation layer which comprises incorporating in gelatin having an ash content less than about 0.2% and having its pH adjusted with only an organic alkali, a compound of the general formula:



where R and R' represent the atoms necessary to complete a ring structure and X represents an alkali metal radical and coating the solution on a support.

7. The method of forming a photographic antihalation layer which comprises incorporating murexide in gelatin having an ash content less than about 0.5% and having its pH adjusted with only an organic alkali, and coating the solution on a support.

8. The method of forming a non-halation photographic element, which comprises coating on one side of a transparent support a layer of gelatin containing murexide, said gelatin having an ash content of less than about 0.5% and having its pH adjusted with only an organic alkali, and coating a sensitive emulsion layer on the opposite side of said support.

9. A photographic element comprising a support, a sensitive emulsion layer thereon, and a layer of unsensitized gelatin thereon uniformly colored with a compound of the general formula:



where R and R' represent the atoms necessary to complete a ring structure and X represents a metal radical selected from the group consisting of alkali metal radicals, alkaline earth radicals, and nickel.

SAMUEL E. SHEPPARD. 50  
ROBERT C. HOUCK.